

Jan. 28, 1936.

O. F. MARVIN

2,028,911

## PROCESS FOR MAKING TUNGSTEN CARBIDE CASTINGS

Filed March 19, 1932

2 Sheets-Sheet 1



Inventor  
Orrin F. Marvin  
by John Flam  
Attorney

Jan. 28, 1936.

O. F. MARVIN

2,028,911

PROCESS FOR MAKING TUNGSTEN CARBIDE CASTINGS

Filed March 19, 1932

2 Sheets-Sheet 2



Inventor  
Orrin F. Marvin  
by John Flam  
Attorney

## UNITED STATES PATENT OFFICE

2,028,911

PROCESS FOR MAKING TUNGSTEN  
CARBIDE CASTINGSOrrin F. Marvin, Los Angeles, Calif., assignor to  
Mills Alloys, Inc., Los Angeles, Calif., a corpo-  
ration of Delaware

Application March 19, 1932, Serial No. 599,938

4 Claims. (Cl. 22—209)

This invention relates to a production of sharply defined cast bodies from difficultly fusible metals, such for example, as tungsten carbide and the like, and more particularly to an improvement 5 over the co-pending application to Oscar L. Mills for a Tungsten carbide product and process of making same, Serial No. 455,732, filed January 17, 1931.

In the above mentioned co-pending application 10 a process is described for producing a cast article of manufacture from molten tungsten carbide which is characterized by a fine grained structure. In this process, a molten tungsten carbide mass is first produced at a temperature above its 15 melting point; as for example, by the aid of the inventions disclosed in the prior patents to Oscar L. Mills, No. 1,718,558, issued July 2, 1929 and No. 1,721,966, issued July 23, 1929. This mass preferably has, by weight, not less than 2 percent of 20 carbon, nor more than 6 percent thereof.

When this material is thoroughly and completely molten, as in a carbon crucible capable of accommodating at least several pounds thereof, it is poured into a mold of the desired 25 configuration, and subjected to pressure for the purpose of securing a fine grain structure. This is accomplished by the aid of centrifugal force; which is produced by providing a rotating mold structure, which in rotating throws the molten 30 material against the walls thereof.

I have found that a uniform and fine grained product can be obtained by the use of a double or combination mold structure, comprising essentially an inner graphite mold proper and an 35 outer mold or support of copper or silver, with the application of pressure, as for example by centrifugal force. This double mold allows the casting to chill slowly enough in order to reduce the possibility of producing internal strains. The 40 graphite shell comprising the mold proper is made so that it retains the heat for a sufficient period to effect this result; and this heat retention property must be enhanced by the aid of further heat insulation, as by an air space, between the copper 45 and the graphite mold. Furthermore, the insulation acts to keep the graphite mold from transferring or absorbing any material amount of heat from the cast alloy, thereby retaining this heat 50 for a long period and preventing unequal or deleterious or partial cooling.

It is a further object of my invention to provide a process for producing sharply defined tungsten carbide articles in commercial quantities, with a minimum expense and expenditure of 55

time, and particularly by casting the article to be formed directly in complete form.

Although I prefer to utilize tungsten carbide without the addition of any other element, a small percentage of free carbon or of other material such as boron, silicon, cobalt, nickel or chromium may be employed, but only to a sparing extent, because such admixtures tend to destroy the copper parts of the mold. Such alloying materials, which of course tend materially to 10 reduce the hardness of the product, are not essential in my process, because I secure the desired structure due to my improved treatment of the molten material.

My invention possesses many other advantages, 15 and has other objects which may be made more easily apparent from a consideration of several embodiments of my invention. For this purpose I have shown a few forms in the drawings accompanying and forming part of the present specification. I shall now proceed to describe these forms in detail, which illustrate the general principles of my invention; but it is to be understood that this detailed description is not to be taken in a limiting sense, since the scope of my invention 20 is best defined by the appended claims.

Referring to the drawings:

Figure 1 is a diagrammatic side elevation of an apparatus utilized in my invention;

Fig. 2 is a fragmentary plan view thereof; 30

Fig. 3 is a fragmentary detailed sectional view of a mold used in practicing my process;

Fig. 4 is a section thereof taken substantially along the plane 4—4 of Fig. 3;

Fig. 5 is a fragmentary detailed sectional view 35 of another form of mold used in practicing my invention;

Fig. 6 is a section thereof taken substantially along the plane 6—6 of Fig. 5; and

Fig. 7 is a front elevation of a cast rotary saw 40 blade formed in the mold shown in Figs. 5 and 6.

In practicing my process, a molten tungsten carbide mass is first produced as by the aid of the invention disclosed by the prior Patents 1,719,558, issued July 2, 1929, and 1,721,966, issued July 23, 45 1929, to Oscar L. Mills. This mass is heated to a temperature above its melting point, and has, by weight, not less than 2 percent of carbon, nor more than 6 percent thereof in the preferred form. It can be alloyed with other metals, but 50 preferably there should not be more than 2 percent by weight of such materials or other impurities. Among such alloying metals may be mentioned the iron group, chromium, molybdenum, tantalum, boron, silicon, thorium and titanium. 55

When the mixture is thoroughly and completely molten, as in a carbon or graphite crucible capable of accommodating at least several pounds of the material, it is poured into a mold of the desired configuration, and subjected to pressure for the purpose of securing a sharply defined product with a fine grain structure. The material is heated to a very high temperature; somewhere in the neighborhood of 5000 to 6000 degrees Fahrenheit, in order to put it in the plastic or fluid state.

I prefer to cast the molten material in a mold that is capable of gradually and uniformly absorbing and transferring the heat from the product. Combination molds having a refractory mold proper made from graphite and an outer surrounding copper or silver jacket or mold are admirably suited for this purpose. Graphite will not materially react with the molten mass and due to its low heat conductivity gradually absorbs and transfers heat away from the product and thus aids in producing the desired casting without internal strains. The thickness of the graphite mold is determined in accordance with the mass of the casting. In general, the larger the casting, the thicker this mold should be.

While the material is still molten, it is subjected to pressure, as hereinabove set forth. A convenient way of accomplishing this is by the aid of centrifugal force. Thus the mold structure can be so arranged that it can be rotated to throw or urge the molten mass against it and in the graphite mold proper to cast the desired sharply defined product.

I have indicated in the present instance a combination mold structure that is capable of casting a product such as a hollow cylinder (Figs. 1-4); however, as will be hereinafter set forth, other sharply defined products can be cast.

The combination mold structure 10 as shown most clearly in Figs. 1-4, comprises an outer shell or mold formed of copper, silver or the like, and an inner graphite mold proper 11.

The outer mold 10 consists of a pair of hollowed out members 12 and 13 which when superimposed in abutting relationship, define a space in which the mold proper 11 resides. There is a mold at each end of the member 10. The mold proper is confined in this space as by a pair of end members 14 formed of graphite, one at each end of member 10. Each of these end members may be provided with inwardly extending corrugations or ribs 15 which cooperate with one end of the mold proper to define air spaces 16' for a purpose and in a manner to be described. A pair of rigid L-shaped metallic end members or brackets 16 and 17 abut against the graphite end members 14 and overlie the ends of the members 12 and 13. The rigid end members 16 and 17 are rigidly secured to the outer mold 10 as by bolts 18 and 19 extending therethrough and into the channel member 13 in order to prevent the graphite end members 14 from becoming displaced or discharged during rotation of the mold. This outer mold, as thus far described, is rigidly secured to a heavy metallic support or base 20 as by bolts 21 and 22.

The top member 12 of the outer mold can be made relatively immovable with respect to the lower member 13 as by a pair of hooks 23. The hooks 23 cooperate with lugs 24 formed on the sides of the top member 12, and the legs thereof extend downwardly through openings 25 in the supporting member 20. A pair of interconnecting levers 26 are pivotally secured at one end to the ends of the legs of the hooks 23 as at 27, and are also pivotally secured at an intermediate point

to a pair of depending lugs 28 formed integral with the base 20. It is apparent that by a single downward movement of the levers 26, the hooks 23 will be lifted upwardly out of engagement with the lugs 24 and permit the relative movement and separation of the top member 12.

The upper member 12 can have a large central aperture 29 to permit the pouring of the molten material into the closed outer mold, which is rotated about a vertical, central axis, in order to throw the material under pressure into the mold proper 11. The pressure thus attained may be of the order of 50 or 200 pounds per square inch, although higher or lower values could be used. The lower member 13 can have a large saucer-like depression 30 in the top face thereof immediately below the aperture 29 in order to permit the molten material poured in to accumulate therein.

The mold proper 11 is adapted to be positioned in the outer mold 10 in the space defined by members 12 and 13, one at each end thereof, although it is readily apparent that more than one can be so positioned by simply changing the inner contour of the outer mold. The mold proper is formed completely of graphite and is shown in this instance as comprising a hollow tubular shell 31 having upstanding end portions or flanges 32 and 33 which abut against the inner periphery of the members 12 and 13. The shell 31 is made of the right thickness to assure a gradual but not too slow cooling of the molten material. In order to prevent the sagging or breaking of this shell, reinforcing wire strands 34 are wound therearound, and a graphite ring 35 is inserted between the shell and the outer mold intermediate the ends of the former. The air space 31' between the shell and outer mold serves as a heat insulation and thus further aids in preventing the quick chilling of the molten mass.

Rear and forward graphite end members 36 and 37 respectively, are inserted in inner peripheral recesses formed in the sleeve 31, and a graphite core 38 extends through these end members and serves to define therewith and with the inner periphery of the shell a space in which the material is to be cast. The end member 36 as well as the flange 32 abut against the tips of the ribs 15 and form with the members 14 the air spaces 16'. These spaces serve as heat insulation spaces to prevent the quick transmission of heat from the mold proper to the copper portions 12, 13.

The forward end member 37 is provided with gates or ports 39 through which the molten material is forced into the space defined by the mold proper upon rotation. Both of the end members 36 and 37 may be provided if desired with central recesses 40 and 41 which provide a space for the formation of bosses on the ends of the cylinder to be cast.

It is apparent that the mold proper 11 is inserted in the outer mold 10 prior to the pouring of the molten material. This can be accomplished by removing member 12 in a manner already outlined.

To provide the above mentioned rotation, I show in this instance a shaft 42 joined to the bottom of the base 20, that can be rotated by any source of motion. For example, in Fig. 1 I show shaft 42 supported in a bracket structure 43 on table 44, and an electric motor 45 conveniently supported under the table, which drives the shaft.

A product, such as a cylinder, formed in the manner above described, is permitted to remain in the mold proper for a short interval of time to permit the gradual and uniform cooling thereof. Usually this interval is attained by the nec-

essary delay incident to the opening of the mold. As hereinabove set forth, the arrangement of a combination mold in the manner and of materials described, assures the gradual, but not too slow, removal of heat from the product. When the product has assumed a self-sustaining form, it is placed in a space where it is still further gradually cooled. This can be accomplished by removing member 12 in the manner described.

10 A space for gradually cooling the product to room temperature can be formed by a box 46 that contains some powdered material that retains heat long enough to insure slow cooling. For example, a mass of silica flour 47 can be used in box 46. If desired, the sides and bottom of the container can be provided with a layer of heat insulating material. This slow cooling effectively prevents internal strains.

Although I have described in detail the formation of a cast tungsten carbide cylinder, my invention is equally applicable to the formation of any desired cast sharply defined body. Thus in Figs. 5-7 a combination mold is shown for the formation of a cast rotary saw blade 48. The 25 mold utilized in making this article is essentially the same both in principle and construction as the mold shown in Figs. 1-4; it differs therefrom merely in the specific construction of the mold proper, for making possible the casting of very 30 thin articles.

The outer mold in this form of the invention, comprises as before, a top and bottom member 12 and 13, end members 16, and base 20. A graphite lining serves as a support and an insulation for the mold proper 52.

35 The graphite lining and support comprises a relatively thick walled hollow tubular member 49 coinciding with the contour of the space defined by members 12 and 13; and an end member 50 closing one end of the tube 49 and positioned adjacent the end metallic members 16. Diametrical- 40 ly opposed slots or grooves 51 are formed in the inner periphery of the tube 49 for the reception of the graphite mold 52.

45 The mold proper 52 comprises two graphite disks 53 and 54 having a diameter substantially equal to the distance across slots 51. A graphite ring 55 of the same diameter as the disks is sandwiched in between the disks, and is provided with

inverse saw teeth 56 on its inner periphery. A core 57 is positioned in a central recess in the disk 53 to provide an opening 59 on the saw blade 48. The disk 53 is formed with ports or gates 58 for the entry of the molten metal into 5 the mold proper 52.

The composite mold thus described is inserted in the slots 51 of the tube 49 and is positioned with its plane surfaces parallel to the longitudinal axis of the tube 49 and the outer mold. In actual 10 practice, the mold proper is first positioned as described, in the tube 49, which is then placed in the outer mold by removing member 12 in a manner already described. The mode of casting is similar to that described in conjunction with the 15 showings in Figs. 1-4. When casting, a large mass of metal is cast around mold 52, in the space between the mold and the cylinder 49. This overlying heavy mass of metal keeps the heat in the mold which would otherwise cool too rapidly. 20 Of course, with larger castings this expedient is unnecessary.

I claim:

1. The process of manufacturing thin castings made from material difficult to fuse, which comprises pouring the fluid material from which the casting is to be made, into a mold and also around the outside of the mold. 25

2. The process of manufacturing thin castings made from material difficult to fuse, which comprises pouring the fluid material from which the casting is to be made, into a graphite mold, and also around the outside of the mold, and maintaining slow heat loss from said poured material. 30

3. The process of manufacturing castings from 35 material having a very high melting point, such as alloys of tungsten carbide, which comprises placing a graphite mold in a massive support so as to be in good heat transferring relation to said support, rotating the support, and pouring the molten material into the support where it is urged by centrifugal pressure into the mold. 40

4. The process of manufacturing castings from material having a very high melting point, such as alloys of tungsten carbide, which comprises 45 subjecting the mold to centrifugal force, and pouring the molten material from which the casting is to be made, in and around the mold.

ORRIN F. MARVIN.